

Patented Dec. 18, 1928.

1,695,337

# UNITED STATES PATENT OFFICE.

FREDERICK C. LANGENBERG, OF WATERTOWN, MASSACHUSETTS, ASSIGNOR TO E. F. HOUGHTON AND COMPANY, OF PHILADELPHIA, PENNSYLVANIA, A CORPORATION OF PENNSYLVANIA.

## CARBURIZER.

No Drawing.

Application filed March 22, 1927. Serial No. 177,469.

My invention relates to that class of compounds known as carburizing or case hardening materials.

One object of my invention is to provide 5 a new and improved compound which is a departure from the usual material used in case hardening or carburizing work.

Another object of my invention is to provide 10 a new type of energizing material which may be used in conjunction with the case hardening or carburizing compounds to accelerate or intensify their action, or may be used to render active as carburizers carbonaceous materials such as charcoal or coke 15 which in themselves have little or no case hardening properties.

Another object of my invention is to provide 20 a relatively cheap carburizing activator which can be applied at a minimum cost and which will render the carburizing compound substantially more permanent in its action.

A further object is to provide an improved 25 method of carburizing or case hardening contemplating the use of the new energizing material in case hardening work. Other objects will be apparent upon consideration of the specification and claims.

My invention is characterized by the employment, as a carburizing activator or energizer, of a mixture of two types of salts of 30 the metals which have carburizing properties, that is to say, a mixture of two types of salts of the alkali or alkaline earth groups, particularly sodium, potassium, barium or calcium, hereinafter referred to throughout the specification and claims as "carburizing" oxides or metals. One of the two types of salts which go to make up the mixture here contemplated comprises the salts of the organic 35 acids, such salts being typified by the formate, acetate, oleate, oxalate, citrate, tartrate and the like. The other type of salt to be used in conjunction with the salts of the organic acids comprises those salts of the alkali or alkaline earth metals whose acid radical 40 contains oxygen and nitrogen, for example the nitrates or nitrites. The salt mixture may be added to a compound having in itself certain carburizing properties, in which case, the addition of the salt will materially 45 intensify and accelerate the carburizing action as well as increase its effectiveness in subsequent runs. The salt mixture may be added to a relatively inert compound, such as coke or charcoal grain, in order to give

carburizing action to it. In this latter case, the resulting compound will be even more effective than the present carburizers of commerce.

The chemical reason for the remarkable 50 action of these salt mixtures as activating and energizing materials is not understood. The presence of the nitrogen oxides together with the carbon dioxide and carbon monoxide freed from the organic salts undoubtedly 55 plays some part and probably the finely divided condition of the alkali or alkaline earth oxides resulting from the liberation of the gases from each molecule of salt aids materially. As hereinbefore pointed out, how- 60 ever, the exact reason is not understood and this chemical discussion is merely theory and is to be considered as such and not in any way binding upon the invention, which broadly 65 comprises the use as carburizing or energizing 70 material of the salt mixture hereinbefore described. However, it is a fact that when these two types of salts are used conjointly, a result will be obtained which will be a 75 striking improvement over the use of any 80 single salt of the classes described.

As hereinbefore pointed out, this new salt mixture may be used as an activator in conjunction with other well known activators, such as sodium, calcium or barium carbonate, 85 to increase the activity and to lengthen the life of the carburizer, or it may be added to the base carbon grains, such as charcoal or coke, in order to render them active as carburizers. In either case, the salt mixture may 90 be added to the charcoal or coke grains in a wide variety of ways with good results. It is to be understood also that more than one of each of the salt types may be added at the same time, if desired. 95

The new activating mixture may be mechanically tumbled in a powdered condition with the grains to be activated until the energizer permeates the grains or becomes frictionally adherent thereto. In this operation, 100 if it is desired, other carburizing compounds may be added to the tumbler. After the tumbling of the grains with the powdered material, a binder such as black strap molasses or hydrocarbon oil may be added to prevent the energizer from dusting off in transit and in use, and the grains may then be treated with a powdered material such as charcoal dust to prevent them from caking. The grains to be activated may be treated with the binder prior 105 110

to the treatment with the energizer and dust or simultaneously with the binder.

With those compounds which are soluble, the energizer may be dissolved in water and the carbonaceous grains immersed therein until the solution has been absorbed. This method provides a means for thoroughly impregnating the grains, thus insuring a permanency in action which is otherwise impossible. After the absorption, if the energizer is to be used with other compounds, the grains can be treated with other energizers such as the powdered carbonates in any well known manner.

15 Further methods of forming the carburizer will be evident to one skilled in the art, for example, a paste of carbonates, formed by moistening them with a saturated solution of the new compound, might be smeared upon the surface of the carbonaceous grains.

16 The percentage of the salts in the mixture will depend on the nature of the material to which it is applied and the work for which the carburizer is intended. Ten per cent or even more of each class may be used successfully to render active a relatively inactive carbonaceous grain, while five per cent or less will serve to greatly intensify the action of a carburizing compound. Even a salt mixture comprising one quarter of one per cent of each salt is sufficient at times to show marked improvement in the action of a carburizing compound, or to render active inert carbonaceous grains.

17 A carburizing material was tested under certain conditions and the depth of total case was measured. Percentages of the salt mixture were added to the compound and comparable tests run to ascertain the increase in depth. The following results are merely indicative of the general effect of the case of these activators and depend on many factors. For this reason, they must not be considered entirely comparable either to each other or to the results obtained with the same percentages of compounds using different conditions of operations. The percentages given are for the increases in the carburizing activity obtained over that of the original carburizer without the addition of the salt mixture:

| Compound added                           | Percentage increase over original depth |
|------------------------------------------|-----------------------------------------|
| 3% calcium acetate, 2% potassium nitrite | 52.8%                                   |
| 3% calcium acetate, 2% sodium nitrite    | 30.2%                                   |
| 3% calcium acetate, 2% strontium nitrate | 28.3%                                   |
| 2% calcium acetate, 3% potassium nitrate | 18.9%                                   |

60 While these figures are given for calcium acetate, corresponding results are obtained with barium oxalate and other organic salts. Other salts of the nitrates and nitrites also give satisfactory results, for example barium and calcium salts have proved to be excep-

tionally applicable. The carburizing material used in the above examples was finely divided spent bone. The first run in each case was made with the carburizer per se while in the second run the spent bone had been impregnated with the given percentages of the compounds. The steel which analyzed carbon .22%, manganese .52%, silicon .235%, sulphur, .012%, phosphorous .01%, nickel .09%, chromium .91%, and vanadium .15% was kept at a carburizing temperature of 925° C. for five and three-fourth hours.

70 Obviously, also, a product containing the essential ingredients of the carburizer may be obtained by other processes, and the invention is not to be limited to any particular process of manufacture. Nor is there any limitation in the proportions of these ingredients in the product, since these may be largely varied to suit the particular work for which the carburizer is intended.

75 I claim:

1. A carburizing material having therein an organic oxygen-containing salt of a carburizing oxide and a salt of a carburizing oxide having nitrogen and oxygen in the acid radical.

80 2. A carburizing compound comprising carbonaceous material, an organic oxygen-containing salt of a carburizing oxide and a salt of carburizing oxide having nitrogen and oxygen in the acid radical.

85 3. A carburizing compound comprising carbonaceous material, an organic oxygen-containing salt of an alkaline earth metal and a salt of a carburizing oxide having nitrogen and oxygen in the acid radical.

90 4. A carburizing compound comprising carbonaceous material, an organic oxygen-containing salt of an alkaline earth metal and a salt of an alkali metal having nitrogen and oxygen in the acid radical.

95 5. A carburizing compound comprising carbonaceous material, an organic oxygen-containing calcium salt and a potassium salt having nitrogen and oxygen in the acid radical.

100 6. A carburizing compound having therein carbonaceous material, calcium acetate and potassium nitrite.

105 7. A carburizing compound having therein charcoal, calcium, acetate and potassium nitrite.

110 8. A carburizing compound having therein charcoal, 3% of calcium acetate and 2% of potassium nitrite.

115 9. A carburizing compound comprising charcoal, a carburizing carbonate, an organic oxygen-containing salt of a carburizing oxide and a salt of a carburizing oxide having nitrogen and oxygen in the acid radical.

120 10. A carburizing compound comprising charcoal, barium carbonate, calcium acetate and potassium nitrite.

125 11. A carburizing material having therein

an organic oxygen-containing salt of a carburizing oxide and a salt of a carburizing oxide having nitrogen and oxygen in the acid radical, the percentage of each substance being present in amounts between  $\frac{1}{4}$  of 1% and 10%.

12. A carburizing material having therein an organic oxygen-containing salt of a carburizing oxide and a salt of a carburizing

oxide having nitrogen and oxygen in the acid radical, the percentage of each substance being present in amounts between  $\frac{1}{4}$  of 1% and 3%.

13. A carburizing compound having therein carbonaceous material, approximately 3% of calcium acetate and 2% potassium nitrite.

FREDERICK C. LANGENBERG.